

## 1

2,712,979

### METHOD FOR REDUCING PYROPHORICITY OF URANIUM HYDRIDE POWDER

Thomas R. P. Gibb, Jr., Marblehead, Mass., and William H. Pasfield, Storrs, Conn., assignors, by mesne assignments, to the United States of America as represented by the United States Atomic Energy Commission

No Drawing. Application February 27, 1952,  
Serial No. 273,764

2 Claims. (Cl. 23—14.5)

This invention relates to powders, such as uranium hydride, which are pyrophoric and, more particularly, to a method for reducing the pyrophoricity of such powders.

It is well known that uranium hydride powder is highly pyrophoric, that is, will ignite upon contact with air. Uranium hydride may be produced by subjecting uranium metal to the action of hydrogen in a closed retort heated to a suitable temperature. As the uranium metal becomes hydrided, the hydride separates from the metal in the form of a finely divided powder. When the uranium metal has been completely hydrided, the retort and its contents are cooled to normal room temperature, that is, to about 20° C.

If the retort now should be opened for the purpose of removing the uranium hydride, the latter would come in contact with air and immediately become ignited. Consequently, it has been necessary to replace the hydrogen in the retort by an inert gas, such as argon, and to transfer the uranium hydride from the retort to its place of storage in an inert atmosphere, such as argon. It also had to be maintained in such an atmosphere during storage.

The present invention is based upon the discovery that the pyrophoricity of uranium powder is reduced so that it can be handled safely in air if the powder has been in contact with the vapor of triethylamine at normal room temperature. Other compounds effective for this purpose are basic organic compounds selected from the group consisting of the other aliphatic amines in which the ratio of the number of carbon atoms to the number of nitrogen atoms is not greater than about six, such as trimethylamine, and aliphatic ethers in which the ratio of the number of carbon atoms to the number of oxygen atoms is not greater than about six, such as diethyl ether, dimethyl ether, ethyl methyl ether, etc. By the term "basic organic

## 2

compound," we mean an organic compound having a free pair of electrons (usually on the oxygen or nitrogen atom) which it can use in a dative type bond with certain other compounds.

5 One method for reducing the pyrophoricity of uranium hydride powder so it can be handled safely in air, therefore, comprises bringing the uranium hydride powder in contact with the vapor of a basic organic compound of the type above mentioned, preferably, at normal room temperature, that is, at a temperature not greater than about 20° C., for a suitable period of time. The period of time required for optimum results varies from a few seconds to between two and three hours depending upon the volatility of the organic basic compound used. An alternative method comprises treating the powder with the basic organic compound in liquid form and then permitting the liquid to evaporate, preferably, at room temperature.

Our investigations have been limited to the treatment of 20 uranium hydride and cerium hydride but we believe the invention may be applicable for treating other metal hydride powders which normally are pyrophoric.

The invention is illustrated further by the following 25 specific example. A thin layer of uranium hydride powder was placed in the bottom of a small test tube in a dry box in an atmosphere of argon. A few drops of triethylamine were placed on absorbent cotton and the cotton wedged into the tube above the powder. After about two and one-half hours, the test tube was removed from the dry box and the cotton was removed from the tube. The uranium hydride powder then was poured from the tube in air upon a concrete surface and the powder was rubbed with the bottom surface of the test tube without ignition of the powder.

30 35 We claim:

1. The method for reducing the pyrophoricity of 40 uranium hydride powder which comprises bringing in contact with the powder the vapor of an aliphatic amine in which the ratio of the number of carbon atoms to the number of nitrogen atoms is not greater than six.

2. The method for reducing the pyrophoricity of 45 uranium hydride powder which comprises bringing the vapor of triethylamine in contact with the powder.

#### References Cited in the file of this patent

Newton et al., Nucleonics, vol. 4, No. 2, February 1949, pages 17-24 at p. 22. (Copy in Scientific Library.)